

# United States Patent [19]

Haberling et al.

[11] 3,850,621

[45] Nov. 26, 1974

[54] HIGH-SPEED TOOL STEELS

[75] Inventors: **Edmund Haberling; Heinrich Kiesheyer**, both of Krefeld; **Hanshermann Weigand**, Tonisvorst, all of Germany

[73] Assignee: **Deutsche Edelstahlwerke Gesellschaft mit beschränkter Haftung**, Krefeld, Germany

[22] Filed: Dec. 26, 1973

[21] Appl. No.: 428,312

[30] Foreign Application Priority Data

Dec. 27, 1972 Germany..... 2263576

[52] U.S. Cl. .... 75/126 A, 75/126 C, 75/126 E, 75/126 H, 75/126 J, 75/126 Q

[51] Int. Cl. .... C22c 39/14

[58] Field of Search ..... 75/126 A, 126 C, 126 E, 75/126 H, 126 J, 126 Q

[56] References Cited

UNITED STATES PATENTS

2,241,187 5/1941 De Vries..... 75/126 Q

3,295,966 1/1967 Steven ..... 75/126 Q  
3,809,541 5/1974 Steven ..... 75/126 A

Primary Examiner—L. Dewayne Rutledge

Assistant Examiner—Arthur J. Steiner

Attorney, Agent, or Firm—Cushman, Darby & Cushman

[57] ABSTRACT

A high-speed tool steel possessing high wear resistance combined with good ductility and machinability, consisting essentially of 0.8 to 1.8 percent carbon, 3.5 to 10 percent chromium, 1 to 13 percent tungsten, 1-10 percent molybdenum, 0.5 to 5 percent vanadium, 0 to 10 percent cobalt, balance iron, wherein the silicon content is not less than 0.5 percent and is determined by the formula:

$$\% \text{ Si} = 2.7 (\% \text{C}) - 0.1 (\% \text{W}) - 0.14 (\% \text{Mo}) - 0.5 (\% \text{V}) + 0.3.$$

3 Claims, 3 Drawing Figures

PATENTED NOV 26 1974

3,850,621



Fig. 1

0.28% Si



Fig. 2

1.07% Si



Fig. 3

2.82% Si

500:1

## HIGH-SPEED TOOL STEELS

This invention relates to high-speed steels having a high wear resistance combined with good machinability and ductility, and particularly relates to such steels wherein the silicon content is a function of the C/W/Mo/V content.

High-speed tool steels are characterized by high resistance to wear up to working temperatures of 600°C. They owe this property to a martensitic matrix which retains its hardness and in which hard carbides formed by ledeburitic solidification are embedded.

It is known that wear resistance can be improved by increasing the proportion of hard carbides in the structure. This feature has hitherto been exploited by using higher vanadium contents up to 5 percent, and higher corresponding percentages of carbon. Although such steels are highly wear-resisting, their high content of coarse particles of vanadium carbide, which has a hardness of about 3000 Vickers, makes them difficult to grind and also reduces their toughness.

Recently the carbide content, and hence the wear resistance, has been raised by increasing the carbon content. Examples embodying such practice are the steels which in the AISI designation are known as M 41 and M 45, and which have vanadium contents of 1 to 2 percent with carbon contents between 1.1 and 1.2 percent. However it has been found that an increase in carbon leads to the development of spiculate carbides of the type  $M_2C$ , instead of the usual high-speed steel carbide  $M_6C$  (DEW Technical Reports 12, 1972, pp 111/33), and their hardness of around 2000 Vickers and unfavourable shape also adversely affect grindability and ductility.

The present invention is directed to solving the problem of producing high-speed tool steels which combine high wear resistance with good grindability and ductility.

The present invention is based on the surprising discovery that provided certain alloying relationships are observed, namely in correlating the silicon content to

completely decomposes in a peritectoid reaction to the MC and  $M_6C$  carbides which then appear in the desired form and distribution.

The invention provides a high-speed tool steel possessing high wear resistance combined with good ductility and machinability, consisting essentially of

|     |        |                 |
|-----|--------|-----------------|
| 0.8 | to 1.8 | % carbon.       |
| 3.5 | to 10  | % chromium      |
| 1   | to 13  | % tungsten      |
| 1   | to 10  | % molybdenum    |
| 0.5 | to 5   | % vanadium, and |
| 0   | to 10  | % cobalt        |
|     |        | balance iron.   |

wherein the silicon content is not less than 0.5 percent and is determined by the formula

$$\% Si = 2.7 (\%C) - 0.1 (\%W) - 0.14 (\%Mo) - 0.5 (\%V) + 0.3$$

By the term "consisting essentially of" in the Specification and claims hereof, is meant that impurities and/or incidental ingredients may be present in the alloys of the invention in such small quantities as not to affect the properties.

The silicon content is thus so adjusted in relation to the percentage contents of the other alloying elements that the formation of undesirable  $M_2C$  carbides is effectively prevented. Any increase in the silicon content above the quantity as hereinbefore set forth leads to an undesirable carbide development and hence to an impairment of the properties of the steel. In such a case coarse primary carbides of the type  $M_6C$  and MC appear.

The content limits of the silicon that is to be introduced according to the present specification are calculated from the equation hereinbefore set forth by reference to the limits in the content ranges of the melting analysis, as hereinafter particularly exemplified.

The compositions of the examined steels within the ranges embraced by the invention are listed in the accompanying Table:

| Steel No. | C    | Cr  | W    | Mo   | V    | Co  | Fe      | Si <sup>+</sup> |
|-----------|------|-----|------|------|------|-----|---------|-----------------|
| 1         | 1.05 | 4.5 | 1.3  | 9.1  | 1.05 | 7.6 | balance | 1.03            |
|           | 1.10 | 5.5 | 1.5  | 9.5  | 1.25 | 8.4 |         | 1.35            |
| 2         | 0.98 | 4.0 | 6.2  | 5.0  | 1.75 | ./. | balance | 0.56            |
|           | 1.03 | 4.5 | 6.5  | 5.25 | 2.0  | ./. |         | 0.89            |
| 3         | 0.98 | 4.0 | 1.5  | 8.0  | 1.75 | ./. | balance | 0.59            |
|           | 1.03 | 4.5 | 1.75 | 8.5  | 2.0  | ./. |         | 0.94            |
| 4         | 0.97 | 5.0 | 2.5  | 2.75 | 2.25 | ./. | balance | 0.97            |
|           | 1.03 | 5.5 | 2.8  | 3.0  | 2.5  | ./. |         | 1.32            |

\* based on the stated content limits of C, W, Mo, V according to the equation as hereinbefore set forth.

the contents of the alloying elements carbon, tungsten, molybdenum and vanadium, the carbide proportion in the structure can be increased without the formation of carbides which by reason of their configuration and hardness impair grindability and ductility. This correlation between the said alloying components according to the invention permits a peritectoid carbide reaction to take place which leads to fine and evenly distributed carbides and hence improves grindability and ductility.

The addition of exactly predetermined quantities of silicon according to the invention enables the carbon content to be raised and so adjusted that although the carbide  $M_2C$  does form during solidification, it is so unstable that upon reheating prior to hot forming it com-

65 The structure of the Steel 1 and of similarly composed steels which differed merely by their silicon contents, containing in one instance 0.26 percent Si more and in the other instance 2.82 percent Si less than the Steel 1 according to the invention, were examined before being worked and also after they had been worked to varying extents.

Reference is made to micrographs illustrated in the accompanying drawings at a magnification  $\times 500$ , of which

65 FIG. 1 shows that the steel containing 0.26 percent Si solidifies with the formation of the spiculate  $M_2C$  carbide and that this remains stable up to high degrees of deformation (FIGS. 1a - c).

FIG. 2 shows that the Steel 1 having a silicon content according to the above formula also solidifies via the  $M_2C$  eutectic but that its carbide is so unstable that this already decomposes as the ingot cools (FIG. 2a). This peritectoid decomposition becomes complete in the course of the following hot working process. Very fine and evenly distributed carbides of type  $M_6C$  and  $MC$  (FIGS. 2b and c) are formed, which impart to the Steel 1 a high resistance to wear coupled with good grindability and toughness.

FIG. 3 demonstrates that silicon contents exceeding that calculated by the equation according to the invention lead to solidification of Steel 1 via the  $M_6C$  eutectic, giving rise to the appearance of coarse primary  $MC$  carbides (FIG. 3a). These coarse carbides cannot be fully broken down even by considerable deformation, and they lead to the development of an irregular coarse-grained structure which adversely affects the properties of the said Steel 1.

The majority of conventional high-speed tool steels have silicon contents that are too low for an optimal development of the carbides. If the present invention is applied to such steels their properties are improved, as illustrated by the following results.

With Steel 2, the plastic bending effort in a static bending test was determined. The Steel 2 had been heat-treated as follows: Hardened by oil quenching from 1,200°C; tempered at 560°C for two periods of one hour. The measured value was 2.5 J. By comparison the corresponding values of steels similar to Steel 2 but containing only 0.3 percent Si and 1.8 percent Si, were about 2 J.

In order to test ductility and cutting performance planing tests were carried out with Steel 3. A tool made of the said Steel 3 was hardened by oil quenching from 1,200°C. and tempered at 550°C. for two periods of one hour. The wear on the underface was measured after 1000 strokes (equivalent to 450 metres total length of cut). The wear in Steel 3 was found to be 0.1 mm. Compared with this result steels similar to Steel 3 but containing 0.3 percent and 1.8 percent Si, showed twice as much wear, viz. 0.2 mm.

In a turning test on blanks made of Steel 4, the durability, i.e., the cutting speed in m/min at which the tool failed, i.e., became useless in 30 minutes' machining, was highest with a time of 19.5 m/min when the silicon content had been adjusted to the contents of the other alloying elements according to the invention. The tools made of Steel 4 were hardened by oil quenching from 1,200°C. and tempered at 540°C. for two periods of one hour. However tests on steels of the composition similar to Steel 4, but in one instance containing 1.8 percent Si, and in another instance 0.3 percent Si, gave V60 durability test results of 19 m/min and 18 m/min.

These tests demonstrate that with compositions according to the relationship of the invention with respect to the silicon content to the carbon, tungsten, molybdenum and vanadium contents, steel having optimum properties is obtained. Increased silicon contents lead to greater hardness but they cause a shift of the secon-

dary hardness maximum to lower annealing temperatures. This reduction in temper stability due to the silicon is a disadvantage in the use of such steels. It has been found that this disadvantage may be overcome by means of further alloying procedures and that the reduction in temper stability due to the silicon can be improved by raising the chromium content of the steels which is normally about 4 percent to higher values.

Thus in a preferred embodiment of the invention the optimum chromium content to ensure stability to temper should be related to the silicon content of the steel by the formula

$$\% Cr = 4 + 2 (\% Si).$$

Silicon additions reduce the residual austenite which is present after the steels have been hardened. In order to mitigate this effect it is therefore advantageous to introduce into silicon-containing steels according to the invention nitrogen up to 0.1 percent.

The present invention enables high-speed tool steels of optimum structure and hence of outstanding applicational properties, such as toughness, wear resistance and grindability to be produced. Despite their improved wear resistance steels composed as proposed by the present invention surprisingly still prove to be readily grindable. Whereas with grinding steels of corresponding other compositions the grinding wheels quickly choked and became blunted causing inadmissible heating and scorching of the ground tools, steels of the proposed composition could be ground substantially without any difficulty.

High-speed tool steels according to the invention are particularly suitable for the making of tools which call for a considerable amount of grinding to give them their final shape, particularly twist drills, taps, cutters, reamers and milling tools.

What is claimed is:

1. A high-speed tool steel possessing high wear resistance combined with good ductility and machinability, consisting essentially of

|     |        |               |
|-----|--------|---------------|
| 0.8 | to 1.8 | % carbon,     |
| 3.5 | to 10  | % chromium,   |
| 1   | to 13  | % tungsten,   |
| 1   | to 10  | % molybdenum, |
| 0.5 | to 5   | % vanadium,   |
| 0   | to 10  | % cobalt,     |
|     |        | balance iron, |

50 wherein the silicon content is not less than 0.5 percent and is determined by the formula

$$\% Si = 2.7 (\% C) - 0.1 (\% W) - 0.14 (\% Mo) - 0.5 (\% V) + 0.3.$$

55 2. A high-speed tool steel according to claim 1, wherein the chromium content is adjusted by reference to the silicon content according to the formula

$$\% Cr = 4 + 2 (\% Si).$$

3. A high-speed tool steel according to claim 1, 60 wherein it contains up to 0.1 percent nitrogen.

\* \* \* \* \*